

[54] PETROLEUM MIDDLE DISTILLATE FUEL  
WITH IMPROVED LOW TEMPERATURE  
FLOWABILITY

[75] Inventor: Nicholas Feldman, Woodbridge,  
N.J.

[73] Assignee: Exxon Research and Engineering  
Company, Linden, N.J.

[22] Filed: June 4, 1973

[21] Appl. No.: 366,537

Related U.S. Application Data

[63] Continuation-in-part of Ser. No. 157,615, June 28,  
1971, abandoned.

[52] U.S. Cl. .... 44/62, 44/63, 44/70,  
44/71, 44/72

[51] Int. Cl. .... C10I 1/22

[58] Field of Search .... 44/62, 63, 70, 71, 72

[56] References Cited

UNITED STATES PATENTS

3,250,599 5/1966 Kirk et al. .... 44/62

|           |         |                      |       |
|-----------|---------|----------------------|-------|
| 3,444,082 | 5/1969  | Kautsky .....        | 44/62 |
| 3,645,704 | 2/1972  | Burkard .....        | 44/62 |
| 3,676,089 | 7/1972  | Morris .....         | 44/62 |
| 3,288,577 | 11/1966 | Patinkin et al. .... | 44/62 |
| 3,337,313 | 8/1967  | Otto .....           | 44/62 |

Primary Examiner—Daniel E. Wyman

Assistant Examiner—Mrs. Y. H. Smith

Attorney, Agent, or Firm—Byron O. Dimmick

[57] ABSTRACT

The low temperature flowability of a middle distillate petroleum fuel boiling within the range of about 250° and about 700°F. at atmospheric pressure is improved by adding to the fuel a combination of a microcrystalline petroleum wax and a wax modifying additive which comprises either a polymer containing halogenated polymethylene segments or an N-aliphatic hydrocarbyl succinamic acid or a derivative thereof. The invention is particularly advantageous in improving the flow of a diesel fuel through a fine filter at low temperatures.

9 Claims, No Drawings

**PETROLEUM MIDDLE DISTILLATE FUEL WITH  
IMPROVED LOW TEMPERATURE FLOWABILITY  
CROSS REFERENCE TO RELATED APPLICATION**

This application is a continuation-in-part of application Ser. No. 157,615, filed June 28, 1971 now abandoned.

**FIELD OF THE INVENTION**

Heating oils and other middle distillate petroleum fuels, e.g., diesel fuels, contain normal paraffin hydrocarbon waxes which, at low temperatures, tend to precipitate in large crystals in such a way as to set up a gel structure which causes the fuel to lose its fluidity. The lowest temperature at which the fuel will still flow is generally known as the pour point. When the fuel temperature goes below the pour point and the fuel is no longer freely flowable, difficulty arises in transporting the fuel through flow lines and pumps, as for example when attempting to transfer the fuel from one storage vessel to another by gravity or under pump pressure or when attempting to feed the fuel to a burner. Additionally, the wax crystals that have come out of solution tend to plug fuel lines, screens and filters. This problem has been well recognized in the past and various additives have been suggested for depressing the pour point of the fuel oil. One function of such pour point depressants has been to change the nature of the crystals that precipitate from the fuel oil, thereby reducing the tendency of the wax crystals to set into a gel. Small size crystals are desirable so that the precipitated wax will not clog the fine mesh screens that are provided in fuel transportation, storage, and dispensing equipment. The pour point of a petroleum fuel oil is not the only measure of the flowability of that fuel at low temperatures; an equally important factor is the low temperature filterability of the fuel, i.e., its ability to pass through a filter. It is thus desirable to obtain not only fuel oils with low pour points, but also oils that will form small wax crystals so that the clogging of filters will not impair the flow of the fuel at low operating temperatures.

**DESCRIPTION OF THE PRIOR ART**

It is known in the prior art to employ various polymeric and copolymeric materials as pour point depressants for wax-containing petroleum fractions. Chlorinated polymers of ethylene are taught for this purpose in U.S. Pat. No. 3,337,313. The use of an alkenyl succinamic acid that is disubstituted on the nitrogen atom or of the amine salts of such acids, and the use of such acids or their salts in combination with a low molecular weight ethylene-olefin copolymer are taught in U.S. Pat. No. 3,444,082. The use of a combination of a petroleum microcrystalline wax and certain pour point depressant additives including copolymers of olefins and styrene, condensation products of naphthalene and sperm oil, or copolymers of ethylene and vinyl acetate is taught in U.S. Pat. Nos. 3,250,599 and 3,288,577. The surprisingly effective combinations of microcrystalline wax with the additives used in the present invention are not disclosed in the prior art.

**DESCRIPTION OF THE INVENTION**

In copending application Ser. No. 157,615 of which the present application is a Continuation-In-Part, it is taught that the low temperature flow properties of a

middle distillate fuel can be improved by incorporating a combination of an amorphous hydrocarbon fraction, substantially free of normal paraffinic hydrocarbons, and either a polymer containing halogenated polymethylene segments or an N-aliphatic hydrocarbyl succinamic acid or a derivative thereof. It has now been surprisingly found that the low temperature flow properties of a petroleum middle distillate fuel oil can be improved by incorporating, in combination with either

5 the above-described halogenated polymer or the N-aliphatic hydrocarbyl succinamic acid, a small quantity of a microcrystalline wax that contains appreciable quantities of normal paraffinic hydrocarbons. More specifically there are added to a waxy middle distillate 10 petroleum fuel from about 0.05 to about 2.5 wt. percent of a microcrystalline wax and from about 0.005 to about 0.5 wt. percent of a fuel-soluble additive component selected from the group consisting of a halogenated ethylene-containing polymer with a halogen content of from about 1 to 40 wt. percent and an alkenyl 15 succinamic acid material, both of which are more fully described below.

The distillate fuel oils that can be improved by this invention include those having atmospheric boiling 20 ranges within the limits of about 250°F. to about 700°F. The distillate fuel oil can comprise straight run or virgin gas oil or cracked gas oil or a blend in any proportion of straight run and thermally and/or catalytically cracked distillates.

25 The most common petroleum middle distillate fuels are kerosene, diesel fuels, jet fuels and heating oils. Since jet fuels are normally refined to very low pour points, there will generally be no need to apply the present invention to such fuels. The low temperature flow problem is most usually encountered with diesel fuels and with heating oils. A representative heating oil specification calls for a 10 percent distillation point no higher than about 440°F., a 50 percent point no higher than about 520°F., and a 90 percent point of at least 30 35 40

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9

tum containing larger amounts of oil, e.g., 5 to 30 percent oil.

As already stated, one type of pour point depressant additive that is employed in conjunction with a microcrystalline wax in the practice of the present invention comprises an oil-soluble polymer containing halogenated polymethylene segments. This polymer is an oil soluble, halogenated, predominantly hydrocarbon material having an average molecular weight of from about 200 to about 500,000, more preferably from about 500 to 50,000. Most advantageously molecular weights are within the range of about 500 and 10,000. The average molecular weights of the polymers may be conveniently determined by means of an ebullioscope or by means of an osmometer.

The polymers that are halogenated for use in this invention are polymers of ethylene or copolymers of ethylene with other monoolefins of from 3 to 6 carbon atoms, although higher olefins in the copolymers are not excluded. Preferably, the polymer or copolymer contains from 5 to about 100 wt. percent of ethylene.

Preferably the halogenated polymers used in this invention are chlorinated polymers. The chlorination produces chlorine substituents on the polymer chain. The chlorination can be carried out by any one of several procedures, the chlorination progressing until the desired content of chlorine is reached. The optimum chlorine contents will be dependent somewhat upon the particular polymer being chlorinated. Usually the chlorinated materials will contain from about 0.2 to about 40 percent by weight, preferably 1 to 35 percent by weight and most preferably 1.5 to about 25 wt. percent of chlorine.

In one process for chlorinating a polymer, chlorine is bubbled through the molten polymer under temperature conditions within the range of about 150° and 400°F. A second process involves bubbling chlorine through the polymer suspended in an inert solvent, such as carbon tetrachloride (or other chlorinated methanes, chlorinated ethanes, and the like) under temperature conditions of at least 75°F. The rate of reaction may be accelerated by using an actinic light source. In a third process chlorine is bubbled through an aqueous suspension of the polymer. The first two processes are preferred since it is believed that in their use the chlorine contacts a greater portion of the inner polymer chain. It is to be understood that the chlorine addition includes the use of known chlorinating compounds such as sulfonyl chloride, oxalyl chloride, phosphogene and the like.

In general, the polymers and techniques of chlorination most preferred are similar to those used in and described in U.S. Pat. No. 3,337,313, which is incorporated herein by reference in its entirety. One significant difference in the description in that patent is that polymers made by the Ziegler process are equally applicable for use in the present composition. Descriptions of polymerizations and polymers resulting from Ziegler type catalysts suitable for use in this invention will be found in the profuse publications in the art. U.S. Pat. No. 3,389,087 and U.S. Pat. No. 3,474,157 are representative examples of these.

As stated earlier, a second type of pour point depressant additive employed with the microcrystalline wax in the practice of the present invention comprises an aliphatic hydrocarbyl succinamic acid or a derivative

thereof. The hydrocarbyl succinamic acid can for the most part be represented by the following formula:



wherein R is a straight chain aliphatic hydrocarbon group having either 0 or 1 site of olefinic unsaturation (alkyl or alkenyl) attached at a secondary carbon atom to the succinyl group and is of at least 14 carbon atoms, generally in the range of 15 to 40 carbon atoms and more usually in the range of 15 to 30 carbon atoms. One of X and X<sup>1</sup> is hydroxyl and the other is:



wherein N has its normal meaning of nitrogen and Y and Y<sup>1</sup> are aliphatic hydrocarbyl groups of from 14 to 40 carbon atoms, more usually of from 15 to 30 carbon atoms, the total of Y plus Y<sup>1</sup> being from about 30 to 52 carbon atoms, more usually from 32 to 48 carbon atoms, and, preferably, from 32 to 40 carbon atoms.

Y and Y<sup>1</sup> can be aliphatically saturated or aliphatically unsaturated, generally free of acetylenic unsaturation (i.e., either alkyl or alkenyl). There can be from one to two sites of olefinic unsaturation. Y and Y<sup>1</sup> may be the same or different and may be straight chain or branched chain, preferably straight chain. The branches will normally be not greater than 1 carbon atom, i.e., methyl. The position of attachment to nitrogen can be at a terminal or at an internal carbon atom.

As is evidenced from the above formula, it is not important which position the alkyl or alkenyl group has in relation to the carboxamide or carboxyl group. Because of the bulky nature of the amine, the usual method of preparation through the succinic anhydride will provide the alkenyl group  $\beta$  to the carboxamide as the major product. To the extent that this is the more easily accessible derivative, this derivative is preferred. However, as far as operability is concerned, either isomer or a mixture of the two isomers can be used. Individual compounds or mixtures of compounds may be used. Mixtures of different C- and/or N-substituents, both as to homologs and isomers, will frequently be employed when the individual precursors to the succinamic acid product are not readily available. Illustrative succinamic acids include: N,N-dihexadecyl hexadecylsuccinamic acid; N-hexadecyl, N-octadecyl octadecylsuccinamic acid; N,N-dihexadecenyl, C<sub>15-20</sub>-alkenylsuccinamic acid; N-hexadecenyl, N-eicosenyl octadecylsuccinamic acid; N,N-dioctadecenyl C<sub>16-18</sub>-alkenylsuccinamic acid; etc.

As indicated previously, the succinamic acid may be used as its amine salt, preferably as a mixture of acid and amine salt. The acid or the amine salt or mixtures thereof can be represented by the following formula:



wherein R is as previously defined, and one of the X<sup>2</sup> and X<sup>3</sup> is  $-NYY^1$  wherein Y and Y<sup>1</sup> are as previously defined. The other of X<sup>2</sup> and X<sup>3</sup> is of the formula:



wherein Y<sup>2</sup> and Y<sup>3</sup> may be hydrogen, aliphatic hydrocarbon of from 1 to 30 carbon atoms or oxaliphatic hy-

drocarbon of from 3 to 30 carbon atoms, there being 1 ethereal oxygen atom present in the radical bonded to nitrogen at least  $\beta$  to the nitrogen atom).  $Y^2$  and  $Y^3$  may be taken together to form a heterocyclic ring of from 5 to 7 members having nitrogen and oxygen as the only heteromembers. The value of  $n$  varies from 0 to 1, preferably from 0.1 to 0.9; that is, from 10 to 90 mole percent of the succinamic acid present is in the form of its salt.

The aliphatic hydrocarbon groups are preferably saturated and if unsaturated will usually have no more than 2 sites of ethylenic unsaturation. The total number of carbon atoms for  $HN^1Y^2Y^3$  will be from 0 to 60, usually 1 to 40.

The groups indicated for  $Y$  and  $Y^1$  may also be used for  $Y^2$  and  $Y^3$ . Usually, where an amine other than the one used to prepare the succinamic acid is used to form the salt, as will be explained subsequently, there will be a mixture of salts; both the added amine and the secondary amine employed to prepare the succinamic acid will be involved in salt formation. Primary amines may be used as well as secondary amines to form the salt. Illustrative amines that can be used to form salts include di-sec-butyl amine, heptyl amine, dodecyl amine, octadecyl amine, tert-butyl amine, morpholine, diethyl amine, methoxybutylamine, methoxyhexylamine, etc.

The hydrocarbyl succinamic acids of this invention are readily prepared by reacting an alkyl or alkenyl succinic anhydride with the desired secondary amine at a temperature in the range of about 150° to 250°F. in approximately equimolar amounts, either neat or in the presence of an inert solvent. The time for the reaction is generally in the range of 15 minutes to 1 hour. This reaction is well known in the art and does not require extensive discussion here.

The alkyl or alkenyl succinic anhydride that is used may be an individual compound or may comprise mixtures of compounds; that is, various alkyl or alkenyl groups of differing number of carbon atoms or different positions of attachment to the succinic anhydride group may be used. Alternatively, a single isomer may be used. Since mixtures are generally more readily available, to that degree they are preferred. Frequently, use will be made of mixtures of aliphatic hydrocarbyl substituted succinic anhydrides wherein no single homolog is present in amount greater than 25 mole percent, each homolog being present in at least 5 mole percent.

Various secondary amines, both those having the same aliphatic hydrocarbon groups and those having different aliphatic hydrocarbon groups, can be used in making the succinamic acid. Either alkyl or alkenyl substituents may be present on the nitrogen, each having at least 14 carbon atoms. The range of difference between the two aliphatic hydrocarbon groups bonded at the nitrogen is not critical, but will generally be fewer than 8 carbon atoms, more usually fewer than 6 carbon atoms. For the most part, the aliphatic hydrocarbon groups will be straight chain, i.e., normal, with the amino nitrogen bonded either to internal or to terminal carbon atoms.

It has been found that when using approximately a 1:1 mole ratio of amine to succinic anhydride, depending on the reaction conditions, a significant amount of amine may be unreacted and remain to form the salt of the succinamic acid that is formed. In some instances, as much as 30 percent of the amine may remain unreacted, forming a significant amount of salt. Thus, the salt will frequently be from 10 to 30 mole percent of the total succinamic acid present.

Also, in situations where significant amounts of water are present during the course of the reaction, the water may react with a succinic anhydride to form succinic acid. If the temperature is not high enough to regenerate the succinic anhydride, the succinic acid will probably remain unreacted or form the amine salt with available unreacted amine. Therefore, the mixtures of amine acid salts may be conveniently prepared merely by using a 1:1 mole ratio of amine to succinic anhydride, and not attempting to drive the reaction to completion, or up to a mole excess of amine.

The amine salts are readily prepared by adding the amine to the succinamic acid either as such or in an inert solvent. Mild heating may facilitate the reaction.

An optional aspect of this invention is to use, in combination with the succinamic acid component, one or more olefin polymers, particularly ethylene-olefin copolymers of from about 1,000 to 100,000 molecular weight, preferably from about 1500 to 20,000 molecular weight wherein the mole ratio of ethylene to its comonomer is from about 6:1 to about 12:1.

The polymers employed in this aspect of the invention should have polyethylene segments in the polymer approximating the chain length of the wax. That is, the polyethylene segments should have from about 6 to 30 monomers on the average.

Thus the major function of the other monomer is to act as a divider between the polyethylene segments. For this reason, various monomers may be used that can be conveniently copolymerized with the ethylene. Such olefins include hydrocarbon terminal olefins and mixtures thereof of from about 3 to 30 carbon atoms, more usually of from about 10 to 30 carbon atoms and various heteroatom-containing addition polymerizable terminal olefins such as the acrylates, methacrylates, vinyl ethers, vinyl ketones, vinyl esters, dicarboxylic acids and esters, etc.

The hydrocarbon olefins that find use in the copolymers will have the following formula:



wherein  $W$  is hydrogen or methyl and  $Z$  is hydrocarbon of from 1 to 30 carbon atoms, more usually alkyl,  $Z$  is free of aliphatic unsaturation.

For the most part, the heteroatom-containing olefins will have the following formula:



where  $W^1$  is hydrogen, alkyl of from 1 to 3 carbon atoms or  $Z^1$ , and  $Z^1$  is hydrocarboxy carbonyl



where Q has from 1 to 20 carbon atoms and is aliphatically saturated hydrocarbyl, hydrocarbyloxy, acyloxy ( $QCO_2-$ ), or hydrocarbyl carbonyl.  $Z^1$  is free of aliphatic unsaturation.

The preferred  $Z^1$  is acyloxy or hydrocarbyloxycarbonyl. The heteroatom-containing monomer will generally be of from 4 to 24 carbon atoms, more usually of from 4 to 20 carbon atoms, have from 1 to 2 oxygen heteroatoms, and have only one site of olefinic unsaturation as its only aliphatic unsaturation.

The method of preparation of the polymer or copolymer used with the succinamic acid component is not critical to this invention. Any convenient method for obtaining polymers of the desired molecular weight may be used. In preparing the hydrocarbon copolymers, usually nonstereospecific catalysts will be employed. Illustrative of such catalysts are triethylaluminum with vanadium oxychloride or titanium tetrachloride. These catalysts are in the category known as "Ziegler-type" catalysts. Alternatively, free radical, high pressure polymerizations may also be used.

The ratio of alkenyl succinamic acid component to other polymers will generally be about 0.25 to 10 parts of the succinamic acid or salt to 1 part of the polymer, more usually from about 2 to 8 parts of the succinamic acid component per part of polymer, preferably 3 to 6 parts of acid component to polymer.

The fuel compositions of this invention will contain from about 0.01 to about 2.5 wt. percent of the microcrystalline wax and from about 0.005 to about 0.5 wt. percent of the other additive, i.e., the halogenated ethylene-containing polymer or the hydrocarbyl succinamic acid or its amine salt or combination of hydrocarbyl succinamic acid component and olefin polymer or copolymer as hereinabove described. The weight ratio of the two components in the combination can range from about 20:1 to 1:20, more usually from about 10:1 to 1:10 and most preferably from about 5:1 to 1:5. Although the separate components can be blended directly into the fuel by simple mixing it will frequently be found desirable to prepare a concentrate by first associating each component with a separate solvent or by dissolving the two components in a common solvent. For example, heavy solvent naphtha or a similar solvent or aromatic character can be employed. The concentrates can contain from 5 to 60 wt. percent of total additives.

This invention will be further understood when reference is made to the following examples which include preferred embodiments.

#### EXAMPLE 1

Fuel oil blends were prepared using a middle distillate fuel oil consisting of 75 vol. percent of cracked distillates having a final boiling point of 665°F. and 25 vol. percent of straight run heavy virgin naphtha, the fuel oil having a cloud point of +12°F. and an API gravity of 30.1 at 60°F. To separate portions of this fuel oil there were added different percentage concentrations of a microcrystalline wax, and to other portions there were added different percentage concentrations of an alkenyl succinamic acid derivative, or a halogenated substantially ethylene-containing polymer. To still other portions of the fuel oil there were added both the microcrystalline wax and either the alkenyl succinamic acid derivative or the halogenated ethylene-containing polymer.

the microcrystalline wax used in the above blends had a molecular weight of 634, a melting point of 167°F., and a normal paraffin content of 22.6 percent. The halogenated polymer was a substantially ethylene-containing polymer having a number average molecular weight of 2,500 and a chlorine content of 21 weight percent and was otherwise identified as Tolad 33 obtained from the Tretolite Division of Petrolite Company. The succinamic acid derivative was a material 10 known as OFA-410 supplied by the Chevron Chemical Company. The preparation of such succinamic acid is described in Example 1 of U.S. Pat. No. 3,444,082. The Tolad was in the form of a 50 wt. percent concentrate in a hydrocarbon oil, and the OFA-410 was in the form 15 of about 70 wt. percent concentrate in a hydrocarbon oil.

Each of the fuel oil blends as well as a sample of the fuel oil without additives was subjected to a low temperature flow test known as a low temperature screen test, in which a 200 ml. sample of the oil is cooled at a controlled rate of 4°F. per hour until a temperature of -10°F. is reached, this being the temperature at which the flow test is conducted. The oil at the test temperature is caused to flow from an upper compartment of the tester into a lower compartment of the tester, all held at the test temperature, the oil passing by gravity through a 30 mesh screen of 1 centimeter diameter for 25 seconds. The volume percentage of oil that has flowed through the screen at the end of this time is 20 then measured. If more than 90 volume percent of the oil has gone through the screen at the end of the 25 seconds, the oil is considered to have passed the test.

The compositions of the various heating oil blends tested and the test results obtained in the low temperature flow test are given in Table I which follows. The weight percentages of the added materials are based on the total composition in each instance. The stated amount of second additive in each case is that of the concentrate of the respective additive and not of active ingredient.

TABLE I

| Additives Used | Microcrystalline Wax | Second Additive | Percent Oil Passing Through Screen at -10°F. |
|----------------|----------------------|-----------------|----------------------------------------------|
| 45             | None                 | None            | 0                                            |
|                | 0.2 wt. %            | None            | 0                                            |
|                | 0.4 wt. %            | None            | 0                                            |
| 50             | None                 | 0.025% Tolad 33 | 40                                           |
|                | None                 | 0.05% OFA-410   | 45                                           |
|                | 0.2 wt. %            | 0.015% Tolad 33 | 100                                          |
|                | 0.2 wt. %            | 0.025% OFA-410  | 100                                          |

55 The data in Table I show that while the alkenyl succinamic acid derivative and the halogenated ethylene-containing polymer each improved the low temperature properties of the heating oil to some extent, the microcrystalline wax gave no improvement in low temperature flow, and yet the combinations of microcrystalline wax and either of the other additives were very effective in improving the low temperature flow properties of the heating oil.

#### EXAMPLE 2

65 The additive combinations of the present invention were also tested in a diesel fuel wherein the requirements are more severe than for a heating oil since a die-

sel fuel must pass through much finer screens or filters. Blends were prepared in a diesel fuel comprising 45 percent catalytically cracked and 55 percent virgin distillates. The diesel fuel had an atmospheric boiling range of 396° to 646°F., a cloud point of +2°F. and an API gravity of 34.2 at 60°F. The diesel fuel and blends containing the additives were subjected to a low temperature filterability test in which 200 ml. of the fuel is cooled at a rate of 4°F. per hour until a temperature of either -5°F. or -10°F. is reached, these being the temperatures at which the flow test is conducted. The cold diesel fuel is then caused to flow through a 325 mesh screen of 1 centimeter diameter using an applied vacuum of 4 inches of mercury, and the percentage of the fuel flowing through the screen in 25 seconds is determined.

The compositions of the diesel fuel blends tested and the test results obtained are given in Table II which follows. The microcrystalline wax used was the same as that in Example 1.

TABLE II

| Additives           | Percent Diesel Fuel Through |          |           |
|---------------------|-----------------------------|----------|-----------|
|                     | 325 Mesh Screen in 25 Sec.  | At -5°F. | At -10°F. |
| None                | 0                           | —        | —         |
| 0.25% Microwax      | 0                           | —        | —         |
| 0.5% Microwax       | 0                           | —        | —         |
| 0.15% Tolad 33      | 30                          | 20       | —         |
| 0.20% Tolad 33      | 35                          | 25       | —         |
| 0.10% OFA-410       | 55                          | 0        | —         |
| 0.20% Microwax plus | 100                         | 100      | —         |
| 0.05% OFA-410       | 100                         | 100      | —         |
| 0.20% Microwax plus | 100                         | 65       | —         |
| 0.15% Tolad 33      | 100                         | 65       | —         |

It will be noted that the succinamic acid additive improved low temperature flow properties to some extent at -5°F. but did not improve the low temperature flow at -10°F., while the microcrystalline wax did not improve the low temperature flow properties at all, and yet the combination of the succinamic acid derivative and the microcrystalline wax gave a 100 percent recovery of fuel at both -5°F. and -10°F. The combination of 0.1 percent of the chlorinated ethylene polymer and 0.2 percent of microcrystalline wax gave a slightly better improvement than with 1½ times as much of the chlorinated polymer alone.

#### COMPARATIVE EXAMPLE

In the same manner as in Example 2, blends were prepared with the same diesel fuel base as in that example. In one blend there was used a combination of the microwax with a copolymer, of about 2,200 number average molecular weight, of about 60 wt. percent ethylene and 40 wt. percent isobutyl acrylate, referred to below as EBACr. The second blend contained a mixture of the microcrystalline wax and a copolymer of ethylene and vinyl acetate, and the third blend contained a combination of the microwax and a different copolymer of ethylene and vinyl acetate. The one copolymer of ethylene and vinyl acetate, referred to below as EVA-1, contained about 65 wt. percent of ethylene and 35 wt. percent of vinyl acetate and had a number average molecular weight of about 2400. A description of the preparation of this copolymer appears in U.S. Pat. No. 3,600,057, column 5, lines 22-45. The second copolymer of ethylene and vinyl acetate, referred to as EVA-2, had a number average molecular weight of

about 1,900 and a mole ratio of ethylene to vinyl acetate of about 4.2 to 1. A description of the preparation of this copolymer appears in Example 1 of allowed pending application Ser. No. 807,966, filed Mar. 17, 1969. See also Canadian Patent 882,194. A principal difference between copolymers EVA-1 and EVA-2, is that the latter has about 3 methyl-terminating side branches on the polyethylene backbone per hundred methylene groups in the backbone as compared with about 12 such side branches per hundred backbone methylene groups in the EVA-1 copolymer. All three of the copolymer materials described above have been used in commerce as fuel oil pour point depressants. Each of these was used in this example in the form of a hydrocarbon oil concentrate having about 50 wt. percent active ingredient. The microwax was the same as in Example 1.

The blends referred to were subjected to the low temperature filterability test described in Example 2, the test being run at -5°F. The compositions of the blends tested and the test results obtained are given in Table III which follows.

TABLE III

| Additives          | Percent Diesel Fuel Through 325 Mesh Screen in 25 Sec. at -5°F. |    |
|--------------------|-----------------------------------------------------------------|----|
|                    | 30                                                              | 35 |
| 0.2% Microwax      | 0                                                               | —  |
| 0.3% EBACr         | 0                                                               | —  |
| 0.3% EVA-1         | 5                                                               | —  |
| 0.3% EVA-2         | 22                                                              | —  |
| 0.2% Microwax plus | 0                                                               | —  |
| 0.15% EBACr        | —                                                               | —  |
| 0.2% Microwax plus | —                                                               | —  |
| 0.15% EVA-1        | 10                                                              | —  |
| 0.2% Microwax plus | —                                                               | —  |
| 0.15% EVA-2        | 8                                                               | —  |

It is to be noted that in contrast to the combinations of microcrystalline wax and pour point depressant additives coming within the scope of this invention, satisfactory low temperature flow of the diesel fuel through a fine screen did not result with combinations of microcrystalline wax and pour point depressant additive outside the scope of the invention.

The combinations of microcrystalline wax and pour point depressants herein described and claimed may constitute the sole additives that are incorporated in the fuel oil compositions, or they can be employed in conjunction with other additives commonly used in distillate fuels, including rust inhibitors, antioxidants, sludge dispersants, demulsifying agents, dyes, haze suppressors, etc.

What is claimed is:

1. A petroleum distillate fuel having a boiling range within the limits of about 250°F. and about 700°F. which has been improved with respect to its low temperature flow properties by adding thereto:
  - a. about 0.01 to 2.5 wt. percent of a microcrystalline paraffin wax and
  - b. about 0.005 to 0.5 wt. percent of a fuel-soluble additive component selected from the group consisting of:
    - i. a halogenated ethylene-containing polymer having a halogen content of from 1 to 40 wt. percent, and
    - ii. a hydrocarbyl succinamic acid material of the formula:



wherein R is a straight chain aliphatic hydrocarbon having from 0 to 1 site of olefinic unsaturation of from 14 to 40 carbon atoms and attached at a secondary carbon atom to the succinyl group; one of X<sup>2</sup> and X<sup>3</sup> is —NYY<sup>1</sup>, wherein Y and Y<sup>1</sup> are aliphatic hydrocarbyl groups of from 14 to 40 carbon atoms, the other of X<sup>2</sup> and X<sup>3</sup> is of the formula:



wherein n varies from 0 to 1, Y<sup>2</sup> and Y<sup>3</sup> are hydrogen, aliphatic hydrocarbon of from 1 to 30 carbon atoms or oxyaliphatic hydrocarbon of from 1 to 30 carbon atoms, and may be taken together with the nitrogen to which they are attached to form a heterocyclic ring of from five to seven annular members.

2. A fuel composition as defined by claim 1 wherein the proportion of (a) to (b) is within the weight ratio range of from about 20:1 to about 1:20.

3. A fuel composition as defined by claim 1 wherein (b) is a chlorinated homopolymer of ethylene.

4. A fuel composition as defined by claim 1 wherein (b) is a chlorinated copolymer of ethylene and a C<sub>3</sub> to C<sub>6</sub> monoolefin.

5. A fuel composition as defined by claim 1 wherein (b) is a hydrocarbyl succinamic acid material wherein R is derived from mixed C<sub>15</sub>—C<sub>20</sub> cracked wax olefins.

6. A fuel composition as defined by claim 1 wherein said —NYY<sup>1</sup> group is derived from amines selected from the group consisting of:

- a. di(hydrogenated tallow) amine (C<sub>16</sub>—C<sub>18</sub>);
- b. di(behenyl-arachidyl) amine (C<sub>22</sub>—C<sub>24</sub>);
- c. mixtures of the foregoing.

7. A fuel composition as defined by claim 1 wherein said distillate fuel is a diesel fuel.

20

25

30

35

40

45

50

55

60

65

8. An additive combination having the property of improving the low temperature filterability of a petroleum distillate fuel when added thereto which comprises:

- a. a microcrystalline paraffin wax, and
- b. a fuel-soluble additive component selected from the group consisting of:
  - i. a halogenated ethylene-containing polymer having a halogen content of from 1 to 40 wt. percent, and
  - ii. a hydrocarbyl succinamic acid material of the formula:



wherein R is a straight chain aliphatic hydrocarbon having from 0 to 1 site of olefinic unsaturation of from 14 to 40 carbon atoms and attached at a secondary carbon atom to the succinyl group; one of X<sup>2</sup> and X<sup>3</sup> is —NYY<sup>1</sup>, wherein Y and Y<sup>1</sup> are aliphatic hydrocarbyl groups of from 14 to 40 carbon atoms, the other of X<sup>2</sup> and X<sup>3</sup> is of the formula:



wherein n varies from 0 to 1, Y<sup>2</sup> and Y<sup>3</sup> are hydrogen, aliphatic hydrocarbon of from 1 to 30 carbon atoms or oxyaliphatic hydrocarbon of from 1 to 30 carbon atoms, and may be taken together with the nitrogen to which they are attached to form a heterocyclic ring of from five to seven annular members, the weight ratio of component (a) to component (b) ranging from about 20:1 to about 1:20.

9. An additive concentrate comprising from about 5 to about 60 wt. percent of the additive combination of claim 8 in an aromatic hydrocarbon solvent.

\* \* \* \* \*